

## UNITED STATES PATENT OFFICE

RICHARD R. WALTER, OF STARNBERG, GERMANY

## ALLOY OF AZOTIZED CHARACTER

No Drawing. Application filed September 20, 1929, Serial No. 394,136, and in Germany August 5, 1929.

My invention pertains to sintered alloys of the class which include a carbide, a nitride or a carbonitride of a metal or metals of the chromium group and which while hard are also tough by reason of the inclusion of auxiliary metal or metals either from one or more groups and more particularly pertains to an alloy containing azotized, nitrided or nitrified metal from either one, or metals from both, of the iron and chromium groups.

It is known that hard alloys principally consisting of carbides and nitrides or carbonitrides of the chromium group are often manufactured by mixing with lower melting metals of either or both of the iron and chromium groups, pressing of the powdered ingredients and then subjecting them to a sintering process.

The auxiliary metals are purposed to cause the individual particles of the main mass for example, the carbides etc. to stick together as one tenacious piece.

Such alloys find principal use as tools or parts which are subjected to severe wear. However the auxiliary metals, which are in every case softer than the material of the main mass, as for example, the carbides, nitrides etc. reduce the tenaciousness of the alloys against wear or their resistance to wear and it is for that reason that the amount of auxiliary metal to be added is restricted.

It was discovered that this harmful effect of the auxiliary metals can be avoided and their resistance to wear noticeably enhanced if one employs them in the form of azotides i. e. as metals combined with nitrogen. The auxiliary metals of the iron group (Fe, Mn, Ni, Co) or these in combination with metals of the chromium group (Cr, W, Mo, U) are according to this invention first subjected to azotization (in a manner excepting tungsten by itself previously known and suitably by means of dissociated nitrogen while in their powdered condition and before their mixture with the elements to be sintered. In the case of tungsten the azotization requires also the simultaneous presence of hydrocarbons.

I have made the discovery that the nitrification is consummated with markedly greater facility and is also possible with such met-

als which heretofore resisted it, especially with all metals of the iron group (iron, manganese, cobalt and nickel) and of the chromium group (chromium, tungsten, molybdenum and uranium), when the nitrification proceeding follows a superficial carburization or when the carburization occurs simultaneously with the nitrification.

Because the melting temperature generally rises in proportion as the nitrogen content increases, one does not carry the azotization so far as to make the subsequent sintering process more difficult.

It was discovered for instance, that even a content of five-hundredth per cent of nitrogen (.05% N) produces a considerable increase in the tenacity against wear. Expediently one should not use much over one per cent nitrogen (1% N), even though a still greater proportion can be useful, if one reckons with the consequential increase in the temperature required to sinter.

It was also discovered that the azotization of the auxiliary metals need not occur before their mixture with the primary elements, but can also occur with equal success simultaneously during the sintering procedure.

The principal elements like carbides or nitrides or carbonitrides are adequately mixed with the auxiliary metals, as for example, iron, nickel or cobalt and tungsten or others in a powdered state, pressed to formed pieces and these sintered in the usual manner. The azotization then ensues during the sintering process by passage thereover of dissociated nitrogen gas (N) or ammonia (NH<sub>3</sub>) gas or else while one conducts the hydrogen (employed as a protecting gas) through an ammoniacal solution where it becomes charged with ammonia (NH<sub>3</sub>) gas. The formpressed pieces to be sintered, in consequence of their fine porosity, exert a considerable capillary effect to gases and the nitrogen diffuses through the entire cross section of the bodies.

As an example conformable to the invention the following alloy is specified:—seventy percent (70%) tungsten carbide, fifteen percent (15%) azotized tungsten, ten percent (10%) azotized cobalt, three percent (3%) azotized chromium.

I claim:

1. An alloy comprising principally a powdered, pressed and sintered carbonaceous tungsten compound together with at least one homogeneously mixed azotized auxiliary metal of the iron or chromium group.
2. An alloy comprising principally a powdered, pressed and sintered carbonaceous tungsten compound together with homogeneously mixed azotized auxiliary metal of both the iron and chromium groups.
3. An alloy according to claim 1, in which a mixture of azotized tungsten carbide and of an azotized metal of the chromium group is employed.
4. An alloy according to claim 1, in which is employed as auxiliary metal a mixture of azotized metal of the iron group and azotized metals of the chromium group.
5. An alloy comprising over fifty per cent of a carbide of tungsten and azotized auxiliary metals comprising one of the chromium group of higher melting temperature than said carbide and one of the iron group of lower melting temperature than the melting temperature of said carbide, the whole being in powdered, compressed and sintered form.
6. An alloy comprising over fifty (50%) per cent of a carbonaceous compound of metal of the chromium group and the remainder azotized tungsten, azotized cobalt and azotized chromium.

RICHARD R. WALTER.